

June 29, 1926.

1,590,847

L. F. MOORE

BRAKE SHOE ART

Filed Jan. 2, 1926



INVENTOR.  
Lewis F. Moore  
BY Cyrus H. Elmer  
ATTORNEY

## UNITED STATES PATENT OFFICE.

LEWIS F. MOORE, OF ROANOKE, VIRGINIA, ASSIGNOR TO WALKER MACHINE & FOUNDRY CORPORATION, OF ROANOKE, VIRGINIA, A CORPORATION OF VIRGINIA.

## BRAKE-SHOE ART.

Application filed January 2, 1926. Serial No. 78,945.

This invention relates to brake shoes to be applied to brake equipment to engage the wheels of railway cars and railway locomotives.

5 The invention is especially applicable to cast metal brake shoes, the body of the shoe having embedded in it strips or sheets of reinforcing metal, such as wires placed side by side or interwoven or sheet metal per-  
10 forated or reticulated.

The object of this invention is to provide a cast metal brake shoe in which parts are chilled and in which shoe the reinforcing members are effectively brought into en-  
15 gagement or union with the cast metal in all parts of the shoe.

By way of introduction, the construction of my improved brake-shoe, when completed, may be stated as follows. The ends of the  
20 mold in which the brake shoe is to be cast contain metal "chill" blocks or pieces which serve to "chill" and harden the ends of the  
25 brake shoe. This "chilling" involves a relatively rapid cooling of the adjacent molten metal, whereby the time during which the  
30 reinforcing member or members are exposed to the high heat of the molten metal is made relatively short. Furthermore, the manner of pouring the molten metal delivers  
35 the metal into the ends of the mold at less heat than in the intermediate part of the mold. The molten metal is poured into the intermediate part and made to flow thence into the ends. During such flowing a part  
40 of the heat is lost. The other parts of the mold have sand faces which permit slow or prolonged cooling of the adjacent molten metal, whereby the reinforcing material is exposed to the intense heat of the molten metal during a relatively long time. Heretofore it has been found that in the casting of brake shoes containing such reinforcing members and the mold not containing "chilled" blocks, that the reinforcing mem-  
45 ber or members are burned or partially de-  
50 stroyed through the action of the prolonged high heat in the molten metal delivered into the mold. To prevent such burning or partial destroying, the reinforcing members have been coated with a material adapted to resist heat or prevent oxidation of the reinforcing members in the presence of the high heat. It being desirable, for the purpose of making a brake shoe strong and hard and  
55 therefore durable in service, I have "chilled"

the ends of the brake shoes. Before placing the reinforcing members into the mold, I treated them throughout their entire length with a material suited to prevent or much limit oxidation of those members under the prolonged heat present in the mold after the pouring of the molten metal. For such coating, the prior art shows the use of various materials. I have used ground soap stone and mineral oil combined before using. Then I found that oxidizing of the reinforcing members in the part of the shoe not affected by the "chilling" was substantially absent; but I also found that such coating prevents the complete engagement or union of the molten metal with the parts of the reinforcing members embedded in the "chilled" parts of the structure, the coating serving as a separating medium. To allow or cause the reinforcing members to actually reinforce, such complete engagement or union is essential, and to make the brake shoe efficient, it is especially important that the end parts of the shoe be given ample strength by reinforcing. Noting this action of the coating on the parts of the reinforcing members embedded in the chilled end parts of the shoe, I found by experimenting and testing that the imperfect engagement or union between the cast metal and the reinforcing members in those parts of the shoe can be avoided by coating only the parts of the reinforcing members which do not extend into the parts or regions of the structure which are affected by the chilling. On the contrary, by such experimenting and testing it was disclosed that by thus coating the parts of the reinforcing members which were to lie in the region of prolonged heat and not coating the parts of the reinforcing members which were to lie in the regions of short duration of heat, in the finished structure the parts of the reinforcing members which lie in the region of prolonged heat are in the condition previously attained by use of the coating and that the parts of the reinforcing members in the regions of relatively quick cooling were in good condition and were in full and complete engagement or union with those members and the cast metal.

In the accompanying drawings,  
Fig. 1 is a sectional edge elevation of a  
brake shoe constructed according to my in-  
vention;

Fig. 2 is a cross section on the line, 2—2, of Fig. 1;

Fig. 3 is an upright section through one end of a mold used for molding these brake 5 shoes;

Fig. 4 is an upright section on the line, 4—4, of Fig. 3.

Referring to the drawings, A, is a plate metal back. B is the cast metal part of the 10 shoe. C, C are reinforcing members embedded in the cast metal and extending throughout the length of the structure.

Structures like that described in connection with Figs. 1 and 2 have heretofore included the reinforcing members coated with 15 material intended to prevent oxidizing or burning of the reinforcing members, the shoe being cast in molds in which there were no "chilling" members. In the part of the 20 mold shown by Fig. 3, the parts, D, D, are sand and the part, E, is a "chill" block adapted to form parts of the faces at the ends of the mold and bear against parts of the ends of the body formed of the molten metal 25 poured into the mold. Such a chill block is placed into each end of the mold. These chilled blocks make each end of the hot casting a quick cooling part or region extending approximately as far as the line, a—a, in 30 Figs. 1 and 3.

In preparing the reinforcing members for placing them into the mold, the parts between the lines, a—a, are covered or coated with material serving to prevent burning or 35 oxidation of those members, and the parts of said members extending from each line, a—a, to the ends of those members are left without such coating.

When, as above indicated, the reinforcing 40 members thus prepared are placed into the molds and the molten metal is poured into the mold, prolonged cooling of the molten metal and prolonged exposure of the parts of the reinforcing members between the lines, 45 a—a, take place, while in the ends of the molds relatively quick cooling takes place during such a short time as to avoid exposing the adjacent parts of the reinforcing members to such heat as will cause burning or 50 oxidizing of those parts of those members, those members being thus left in condition for complete engagement or union with the cast metal.

It is inferred that when the coating is 55 present on the reinforcing metal and that metal and the coating are exposed to the prolonged heat of the molten metal poured into the mold, the coating is entirely or partially converted and absorbed or neutralized in 60 such manner as to cease to constitute a layer or medium separating the poured metal from the reinforcing metal, and that in the chilling region the heat is not sufficiently intense or prolonged to thus convert and absorb or 65 otherwise eliminate the coating and prevent

it from remaining as a medium separating the reinforcing metal from the poured metal.

In a secondary way, complete engagement between the reinforcing members and the "chilled" ends of the shoes is also important, 70 because even if in service, the end of a shoe fractures, the reinforcing members will prevent the falling of the fractured part to the rail and perhaps cause wrecking. It is well known in railway service that every effort 75 should be made to prevent any part of a brake mechanism from falling so as to be in the way of a wheel. Wrecks of parts of a train and in some cases an entire train have been thus caused. 80

I claim as my invention,

1. A cast metal brake shoe comprising a chilled part and an unchilled part, and reinforcing material embedded in the chilled part and in the unchilled part of the body, 85 the part of the reinforcing material in the unchilled part of the body being coated with heat resisting material and the part of the reinforcing material in the chilled part of the body being bare, substantially as described. 90

2. A cast metal brake shoe comprising chilled ends and an intermediate unchilled part, and reinforcing material embedded in the chilled ends and in said intermediate 95 part and the part of the reinforcing material in said intermediate part being coated with heat resisting material and the part of the reinforcing material in the chilled ends being bare, substantially as described. 100

3. A brake shoe having a cast metal body in which the ends are composed of chilled metal and the part between the ends is composed of unchilled metal, and metal reinforcing embedded in each chilled end and extending into the unchilled metal of the body, the part of the reinforcing in the unchilled part of the body being covered with heat resisting material and the part of the reinforcing in the chilled ends being bare, 110 substantially as described.

4. A brake shoe having a cast metal body in which the ends are composed of chilled metal and the part between the ends is composed of unchilled metal, and metal reinforcing embedded in each chilled end and extending through the unchilled metal of the body, the part of the reinforcing in the unchilled part of the body being covered with heat resisting material and the part of the reinforcing in the chilled ends being bare, 115 substantially as described. 120

5. The herein described method of forming a cast metal brake shoe, which method consists in coating a part of a reinforcing material with heat resisting material and leaving a part of said reinforcing material bare, and then pouring molten metal around the reinforcing material and chilling the molten metal at the part of the reinforcing 125 130

material which is bare and slowly cooling the part of the molten metal surrounding the part of the reinforcing material which is covered with the heat resisting material, substantially as described.

6. The herein described method of forming a cast metal brake shoe, which method consists in coating the middle part of a reinforcing material adapted to extend into the ends and intermediate part of the body of the shoe with heat resisting material and leaving the end parts of the reinforcing material bare, and then pouring molten metal around the reinforcing material and chilling the molten metal at the ends of the molded body and slowly cooling the part of the body intermediate the end parts of the body, substantially as described.

7. The herein described method of making reinforced cast metal brake shoes having chilled ends, which method consists in placing a coating of heat resisting material on the part of the reinforcing material which is to be embedded in the unchilled part of the shoe and leaving the remainder of the reinforcing material bare, and then pouring molten metal around the reinforcing material and rapidly cooling the molten metal on the ends of the shoe and slowly cooling the intermediate part of the molten metal, substantially as described.

In testimony whereof I have signed my name, this 31st day of December, in the year one thousand nine hundred and twenty-five.

LEWIS F. MOORE.